

## UNITED STATES PATENT OFFICE

1,949,682

## NITRIDING

John J. Egan, Brooklyn, N. Y., assignor to Electro  
Metallurgical Company, a corporation of West  
Virginia

No Drawing. Application February 26, 1930,  
Serial No. 431,641

9 Claims. (Cl. 148—16)

My invention relates to the production of nitride cases on ferrous materials by heating the materials in the presence of nitriding agents, and it is the main object of my invention to intensify or accelerate the production of such cases.

Thin, hard, wear-resistant cases on ferrous alloys are useful as wearing surfaces for machine parts. The cases may be produced by nitriding, i. e. by heating the alloys in the presence of nitriding agents to temperatures below the nitride eutectoid temperature at about 600° C. In a nitriding gas, such as ammonia, a treatment of 12 to 20 hours is required to produce the cases, the treating time usually being longer when lower temperatures are used than when higher temperatures are used. The hard, wear-resistant cases are usually produced by heating in an atmosphere of ammonia to about 460° C. to 580° C., the treated alloy containing a promoting agent, such as aluminum or vanadium, which promotes the formation of the hard, wear-resistant coating at these temperatures. By far the most extensive use of my invention is in connection with the production of hard, wear-resistant coatings and the invention will be described with reference thereto.

It has been found that the action of nitriding agents is intensified when a closed chain carbon compound in which nitrogen forms a part of the closed chain is present.

As illustrative of my invention, a specimen of ferrous alloy containing about 95.5% iron, about 1% aluminum, and small amounts of phosphorus, sulphur, manganese, silicon, nickel, molybdenum and carbon was placed in a closed container. Ammonia was bubbled through pyridine which was heated to a temperature just below its boiling point to increase its vapor pressure. The entrapped air in the container was displaced by the mixture of ammonia and pyridine vapor and the container and its contents were heated to 460° C. for 4 hours whilst a slow current of the gas mixture was passed into the container. A thin, uniform, wear-resistant case having a hardness corresponding to about 1000 Brinell was produced on the specimen. A similar hard, wear-resistant case was produced on another specimen of the same alloy when heated for 16 hours without the presence of pyridine vapor. By treatment with ammonia without the pyridine, no appreciable hardness was produced by heating the alloy at 460° C. for 4 hours.

Beneficial results may be produced by the use of other compounds of the above described class as for example, higher molecular weight closed

chain carbon compounds in which at least one nitrogen radical forms a part of a closed chain. Quinoline is such a compound, and is an effective accelerator, and other compounds in which a nitrogen atom occurs in a closed chain may be used.

Any appreciable amount of the accelerator in conjunction with the nitriding agent is sufficient to produce acceleration. The preferred amount to be used with an alloy under given conditions may be determined by experiment for each particular case, but the invention is of course not restricted to the proportion which gives the maximum effect. Considerations of cost make it desirable not to use excessive amounts of the accelerator substance. That is, a modicum of accelerator is generally sufficient.

Although I have given only a few specific examples of accelerators and only one example of a nitriding agent, it is evident that other substances of the classes described may be used and modifications of the described methods may be made without departing from my invention. Therefore, I do not wish to be understood as imposing limitations on my invention except such as are imposed by the prior art and by the annexed claims.

I claim:

1. The method of producing nitride cases on ferrous materials which comprises heating the material at nitriding temperatures below the eutectoid at about 600° C. in the presence of ammonia and an accelerating agent consisting of a closed chain carbon compound in which one nitrogen radical and five carbon radicals form the closed chain.

2. Method of accelerating the production of nitride cases on ferrous materials by heating the materials at nitriding temperatures below the nitride eutectoid at about 600° C. in the presence of ammonia which comprises effecting said nitriding in the presence of an accelerating agent consisting of a closed chain carbon compound in which one nitrogen radical and five carbon radicals form the closed chain.

3. Method of accelerating the production of nitride cases on ferrous materials by heating the materials at nitriding temperatures below the nitride eutectoid at about 600° C. in the presence of ammonia which comprises effecting said nitriding in the presence of an accelerating agent chosen from the group comprising pyridine and quinoline.

4. The method of producing nitride cases on ferrous materials which comprises heating the

60

65

70

75

80

85

90

95

100

105

110

material at nitriding temperatures below the nitride eutectoid at about 600° C. in the presence of ammonia and at least one of the following: pyridine, quinoline.

5. Medium for nitriding ferrous materials comprising ammonia and a modicum of a nitriding accelerator, said accelerator consisting of a closed chain carbon compound in which one nitrogen atom and five carbon atoms form the closed chain; the ammonia predominating over the other constituents of the medium.

6. Medium for nitriding ferrous materials comprising ammonia and a modicum of at least one of the following: pyridine, quinoline; the ammonia forming a preponderating proportion of said medium.

7. Medium for nitriding ferrous materials consisting of ammonia and a modicum of pyridine.

8. The method of producing nitride cases on

ferrous materials which comprises passing ammonia in contact with at least one liquid closed chain compound in which one nitrogen radical and five carbon radicals form the closed chain, whereby a mixture of the ammonia and the compound is formed, and heating the material at nitriding temperatures below the nitride eutectoid at about 600° C. in the presence of the mixture.

9. The method of producing nitride cases on ferrous materials which comprises passing ammonia in contact with at least one compound chosen from the group consisting of pyridine and quinoline, whereby a mixture of the ammonia and the compound is formed, and heating the material at nitriding temperatures below the nitride eutectoid at about 600° C. in the presence of the mixture.

JOHN J. EGAN.

20

80

85

90

95

25

100

30

105

35

110

40

115

45

120